

## UNITED STATES PATENT OFFICE

2,499,807

## PROCESS FOR ELECTROPLATING MOLYBDENUM AND ITS ALLOYS

Leonard F. Yntema, Webster Groves, and Mary Joecile Ksycki, St. Louis, Mo., assignors to president and board of trustees of St. Louis University, St. Louis, Mo.

No Drawing. Application August 31, 1942,  
Serial No. 456,820

9 Claims. (Cl. 204—43)

1

The invention relates to the electrodeposition of molybdenum.

We have discovered that molybdenum may be efficiently electrodeposited from aqueous electrolytes containing molybdic acid, its anhydride or its salts in the presence of aliphatic acids and high concentrations of salts of aliphatic acids.

Among the additional salts which may advantageously be used in our process are the sodium, potassium or ammonium formate, acetate, and propionate or combinations of the same. It is of advantage to employ such concentrations of these salts that the mol ratio of added anion to water is from 1 to 2 up to 1 to 4, preferably between 1 to 2.2 and 1 to 3.

The work on which the electrodeposition of molybdenum is desired is placed in the electrolyte to form the cathode and the anode is a conducting material which will not be attacked by the reaction products at the anode, such as platinum or carbon. A cathode of copper, iron, or nickel has been found to be satisfactory.

The electrolytic bath is preferably maintained slightly acid, the optimum conditions being a pH between 5.5 to 6.8 as measured with a glass electrode. Under some conditions however the pH may be varied from this range and, in particular, a potassium-ammonium propionate bath will give good deposits at a pH of 7.4.

The current density may be varied quite widely but the optimum conditions are between 0.1 to 0.8 ampere per square centimeter of cathode surface. The temperature of the bath is preferably maintained between 30° C. and 50° C.

With our process as above described, we have been able to obtain smooth, bright, adherent deposits of molybdenum in two minutes. The deposited metal is resistant to acids such as cold hydrochloric and sulfuric and is resistant to strong alkalies but is soluble in nitric acid.

Our process is adapted for the electroplating of articles to render them corrosion-resistant as well as to obtain a bright decorative effect. It is useful for preparing molybdenum sheet by obtaining a thick deposit of the metal on a suitable cathode and subsequently dissolving off the cathode leaving the molybdenum in sheet form.

Our process is adapted for the electrodeposition of molybdenum alloys or mixtures with other metals. Iron may be codeposited with molybdenum by adding to the bath a solution of a ferrous salt, such as ferrous sulfate ( $FeSO_4$ ). Cobalt may be codeposited with molybdenum by adding to the bath a solution of a cobalt salt, such as cobalt sulfate ( $CoSO_4$ ). Nickel may be codeposited

2

with molybdenum by adding to the bath a solution of a nickel salt, such as nickel sulfate ( $NiSO_4$ ).

The anions of the aliphatic acids, such as formate, acetate, and propionate, which are present in high concentration increase the solubility of the hexavalent molybdenum compounds in the acid solutions and, with the acid, increase the solubility of reduction products of the hexavalent molybdenum compounds formed during the process of electrolysis, thereby preventing the precipitation of molybdenum hydroxide or of basic salts.

One of the chief advantages of our process is that the molybdenum compounds used are the most readily available compounds of the element. Molybdic anhydride,  $MoO_3$ , and ammonium paramolybdate,  $(NH_4)_5Mo_3O_10 \cdot 4H_2O$  are both commercially available and are both operative in our process.

To illustrate our invention, the following examples are given:

## Example I

An electrolyte is made up of the following composition:

5 g. molybdic anhydride  
60 g. KOH  
55 cc.  $NH_4OH$  (28%  $NH_3$ )  
75 cc.  $HCO_2H$  (87%)  
15 cc.  $H_2O$

Preferably the bath is subjected to a preliminary electrolysis at a current density of 0.5 ampere per square centimeter until the bath becomes red in color. The optimum conditions for obtaining molybdenum from this bath are pH 5.7 to 5.9; current density 0.5 ampere per square centimeter; temperature 30° C. to 40° C. Bright metallic deposits of molybdenum are obtained in five minutes. The weight of an average deposit is 0.5 mg. on an area of 8 square centimeters of cathode surface. The current density range for bright metal plating from this bath is 0.35 to 0.6 ampere per square centimeter.

## Example II

An electrolyte is made up of the following composition:

5 g. molybdic anhydride  
50 g.  $NH_4C_2H_5O_2$   
50 g.  $KC_2H_5O_2$   
10 cc.  $H_3C_2H_5O_2$  (glacial)  
65 cc.  $H_2O$

No preliminary electrolysis is needed. The

## 3

optimum conditions for obtaining deposition of molybdenum from this bath are pH 5.7 to 6.0; current density 0.5 ampere per square centimeter; temperature 30° C. to 40° C. Bright metallic deposits of molybdenum are obtained in two minutes. The weight of an average deposit is 1.0 mg. on 8 square centimeters of cathode surface. The current density range for bright metal plating is from 0.2 to 0.6 ampere per square centimeter.

## Example III

An electrolyte is made up of the following composition:

5 g. molybdic anhydride  
74 cc. prolonic acid ( $\text{HC}_3\text{H}_5\text{O}_2$ )  
32 gm.  $(\text{NH}_4)_2\text{CO}_3$   
19 gm. KOH  
28 cc.  $\text{H}_2\text{O}$

Preferably the bath is subjected to preliminary electrolysis for 15 to 20 minutes at 0.2 ampere per square centimeter. The optimum conditions for obtaining deposition of molybdenum for this bath are pH 6.8; current density 0.2 ampere per square centimeter; temperature 30° C. to 40° C. Bright metallic deposits are obtained in two minutes. The weight of an average deposit is 0.5 mg. on an area of 8 square centimeters of cathode surface. The current density range for bright metal plating from this bath is from 0.15 to 0.4 ampere per square centimeter.

## Example IV

An electrolyte is made up of the following composition:

5 g. molybdic anhydride  
60 g. KOH  
55 cc.  $\text{NH}_4\text{OH}$  (28%  $\text{NH}_3$ )  
75 cc.  $\text{HCO}_2\text{H}$  (87%)  
15 cc.  $\text{H}_2\text{O}$   
30 cc.  $\text{FeSO}_4$  (0.1 M)

The optimum conditions for the codeposition of molybdenum and iron from this bath are a current density of 0.2 ampere per square centimeter; temperature 30° C. to 40° C. Bright metallic plates are obtained in two minutes. The current density range for bright metal plating from this bath is 0.15 to 0.5 ampere per square centimeter.

## Example V

An electrolyte is made up of the following composition:

5 g. molybdic anhydride  
50 g.  $\text{NH}_4\text{C}_2\text{H}_3\text{O}_2$   
50 g.  $\text{KC}_2\text{H}_3\text{O}_2$   
10 cc.  $\text{HC}_2\text{H}_3\text{O}_2$  (glacial)  
65 cc.  $\text{H}_2\text{O}$   
3 cc.  $\text{NiSO}_4$  (0.1 M)

The optimum conditions for obtaining codeposition of molybdenum and nickel from this bath are current density 0.25 ampere per square centimeter; temperature 30° C. to 40° C. Bright metallic plates are obtained in one minute. The weight of an average deposit is 1 mg. on 16 square centimeters of cathode surface. The current density range for bright metal plating from this bath is 0.07 to 1.0 ampere per square centimeter.

## 4

## Example VI

An electrolyte is made up of the following composition:

5 g. molybdic anhydride  
50 g.  $\text{NH}_4\text{C}_2\text{H}_3\text{O}_2$   
50 g.  $\text{KC}_2\text{H}_3\text{O}_2$   
10 cc.  $\text{HC}_2\text{H}_3\text{O}_2$  (glacial)  
65 cc.  $\text{H}_2\text{O}$   
1 cc.  $\text{CoSO}_4$  (0.1 M)

The optimum conditions for the codeposition of molybdenum and cobalt from this bath are current density 0.25 ampere per square centimeter; temperature 30° C. to 50° C. Bright metallic plates are obtained in one minute. The weight of an average deposit is 0.5 mg. on 16 square centimeters of cathode surface. The current density range for bright metal plating from this bath is 0.09 to 0.8 ampere per square centimeter.

The above examples are given by way of illustration only.

What we claim as our invention is:

1. The process of plating metallic molybdenum which comprises passing a current between an anode and the work to be plated as a cathode in an electrolyte comprising an aqueous solution of a compound of the class consisting of molybdic acid, its anhydride and its salts and a high concentration of an anion of an aliphatic acid of the class consisting of formate, acetate and propionate, the ratio of said anion to water being between 1 to 2 and 1 to 4 and the pH being between 5.5 and 6.8.
2. The process of plating metallic molybdenum which comprises passing a current between an anode and the work to be plated as a cathode in an electrolyte comprising an aqueous solution of a compound of the class consisting of molybdic acid, its anhydride and its salts and a high concentration of an anion of an aliphatic acid of the class consisting of formate, acetate and propionate, the ratio of said anion to water being of the order of 1 to 2½ and the pH being between 5.5 and 6.8.
3. An electrolyte for the electrodeposition of metallic molybdenum comprising an aqueous solution of a compound of the class consisting of molybdic acid, its anhydride and its salts and a high concentration of an anion of an aliphatic acid of the class consisting of formate, acetate and propionate, the ratio of said anion to water being between 1 to 2 and 1 to 4 and the pH being between 5.5 and 6.8.
4. An electrolyte for the electrodeposition of metallic molybdenum comprising an aqueous solution of a compound of the class consisting of molybdic acid, its anhydride and its salts and a high concentration of an anion of an aliphatic acid of the class consisting of formate, acetate and propionate, the ratio of said anion to water being between 1 to 2.2 and 1 to 3 and the pH being between 5.5 and 6.8.
5. An electrolyte for the electrodeposition of metallic molybdenum alloys comprising an aqueous solution of a compound of the class consisting of molybdic acid, its anhydride and its salts, a high concentration of an anion of an aliphatic acid of the class consisting of formate, acetate and propionate and a soluble salt of a metal of the class consisting of iron, nickel and cobalt the ratio of said anion to water being between 1 to 2 and 1 to 4 and the pH being between 5.5 and 6.8.
6. The process of electroplating metallic molybdenum which comprises passing a current between an anode and the work to be plated as a cathode in an electrolyte comprising an aqueous

solution of a molybdate compound, an aliphatic acid of the class consisting of formic, acetic, and propionic acids and an alkali salt of an aliphatic acid of the class consisting of formate, acetate and propionate, in which the ratio of the anion of said aliphatic acid and salt of said aliphatic acid to water is between 1 to 2 and 1 to 4, the pH being between 5.5 and 6.8, the temperature being between 30° and 50° C. and maintaining the current density between 0.07 and 1.0 ampere per 10 square centimeter.

7. The process according to claim 6 in which the ratio of the anion of said aliphatic acid and salt of said aliphatic acid to water is maintained between 1 to 2.2 and 1 to 3.

8. The process according to claim 1 in which the anode is a conducting material of the class consisting of platinum and carbon.

9. The process of electroplating metallic molybdenum alloys which comprises passing a current between an anode and the work to be plated as a cathode in an electrolyte comprising an aqueous solution of a molybdate compound, an aliphatic acid of the class consisting of formic, acetic, and

propionic acids and an alkali salt of an aliphatic acid of the class consisting of formate, acetate and propionate, and a soluble salt of a metal to be codeposited with molybdenum of the class consisting of iron, nickel, and cobalt, in which the ratio of the anion of said aliphatic acid and salt of said aliphatic acid to water is between 1 to 2 and 1 to 4, the pH being between 5.5 and 6.8, the temperature being between 30° and 50° C. and maintaining the current density between 0.07 and 1.0 ampere per square centimeter.

LEONARD F. YNTEMA.  
MARY JOECILE KSYCKI.

## REFERENCES CITED

The following references are of record in the file of this patent:

"Quantitative Analysis by Electrolysis," by Classen and Hall, published in 1913 by John Wiley & Sons, Inc., page 146.

"Transactions of the Electrochemical Society," vol. 70 (1936), pages 423, 424.